

1

2,944,900

## SENSITIZATION OF PHOTOGRAPHIC EMULSIONS WITH IONIC POLYALKYENE OXIDE SALTS

Burt H. Carroll, Herbert S. Elins, James L. Graham, and Charles V. Wilson, Rochester, N.Y., assignors to Eastman Kodak Company, Rochester, N.Y., a corporation of New Jersey

No Drawing. Filed Dec. 10, 1956, Ser. No. 627,136

20 Claims. (Cl. 96—100)

The sensitization of photographic emulsions with various onium compounds such as cationic surface-active quaternary ammonium, phosphonium, and ternary sulfonium salts is known as shown by Carroll U.S. Patent 2,271,623 and Carroll and Allen U.S. Patents 2,275,727 and 2,288,226 as well as Carroll and Spence U.S. Patent 2,334,864. The parent invention also shows that emulsions sensitized with the onium compounds can be used in color photography by development of the emulsions with color developing solutions containing coupler compounds which react with color developing agents to form dyes, or the coupler compounds can be present in the emulsions sensitized with the onium compounds.

Similarly, the sensitization of photographic emulsions with various non-ionic polyalkylene oxides such as polyethylene oxide is shown by U.S. Patents 2,423,549 and 2,441,389.

We have discovered that when photographic silver halide emulsions adapted particularly for use in color photography, that is, emulsions containing coupler compounds, are sensitized with non-ionic polyalkylene oxide compounds no improvement in sensitivity occurs or else a loss in light sensitivity of the emulsion is sustained. However, the light-sensitivity of the coupler-containing emulsion is materially increased if instead of using a non-ionic polyalkylene oxide sensitizing agent, the emulsion containing the coupler compound is sensitized with an ionic, i.e. a cationic polyalkylene oxide salt such as a quaternary ammonium or phosphonium polyalkylene oxide salt or a ternary sulfonium polyalkylene oxide salt, e.g. tetraethoxyethyl-bis-pyridinium perchlorate, or an anionic polyalkylene oxide compound such as the carbamic, glutamic and sulfuric acid salts below. This improvement in light sensitivity appears to be independent of the type of developing agent used for developing the emulsion sensitized with the ionic polyalkylene oxide salt, since the sensitivity increase is obtained with both black-and-white developers and color developers. Little else is known of the mechanism involved, but it has been observed that the effect is independent of the type of coupler used in the emulsion since the sensitizing effect is obtained in the presence of either the phenolic hydroxyl or the reactive methylene types of coupler compounds.

While the mentioned sensitivity increase is obtained when employing the polyalkylene oxide salts in coupler-containing emulsions, this sensitivity increase is sometimes accompanied by increase in general fog, particularly upon storage of the emulsions under adverse conditions of temperature and humidity. Therefore, it may be desirable to employ fog reducing substances in the emulsions as illustrated in the examples hereinafter.

It is therefore one object of the invention to provide photographic silver halide emulsions containing coupler compounds which emulsions are sensitized with ionic polyalkylene oxide compounds such as the cationic quaternary ammonium and phosphonium polyalkylene oxide salts, and ternary sulfonium polyalkylene oxide salts and

2

the anionic polyalkylene oxide compounds such as the polyalkylene oxide carboxylic acid salts, polyalkylene oxide bis-N-carboxymethyl carbamate salts, polyalkylene oxide bisulfuric acids, etc. A further object is to provide suitable means for reducing any fog accompanying the use of the ionic polyalkylene oxide salt sensitizers. Another object is to provide color processes utilizing the emulsions thus sensitized. Other objects will appear from the following description of our invention.

10 These objects are accomplished in part by the incorporation of the ionic polyalkylene oxide compounds in photographic silver halide emulsions containing coupler compounds.

The cationic polyalkylene oxide salts used in the emulsions are characterized as containing a bivalent polyalkylene oxide radical such as



and



corresponding to polyethylene oxide, polypropylene oxide and polybutylene oxide radicals to which is attached at least one onium salt group such as a quaternary ammonium, phosphonium or ternary sulfonium salt group, and wherein  $n$  is a positive integer at least as great as 4 representing the least number of alkylene oxide units present in the polyalkylene oxide radical of the salt.

25 The quaternary and ternary polyethylene oxide salts are particularly effective as sensitizers for the emulsions and have the structures



30 in which  $n$  is greater than 3,  $X^-$  is an anion or acid radical such as halide, alkyl sulfate, p-toluenesulfonate or perchlorate, and  $R$ ,  $R_1$  and  $R_2$  are e.g., aliphatic or aromatic radicals such as methyl, ethyl, propyl, benzyl or phenyl.



35 in which  $X^-$ ,  $n$ ,  $R$ ,  $R_1$  and  $R_2$  are as above mentioned, and  $R_4$  is an alkyl or aromatic radical such as methyl, phenyl or p-tert. octylphenyl.

(C) Structures similar to A and B in which N is replaced by



40 in which  $X$  and  $n$  are as above-mentioned and  $Q$  represents the non-metallic atoms necessary to complete an organic heterocyclic nucleus such as pyridyl,  $\alpha$ -picolyl and  $\gamma$ -picolyl.



45 in which  $R_4$ ,  $n$ ,  $Q$  and  $X$  are as above.

50 Representative cationic quaternized and ternarized polyalkylene oxide salts having these formulas are:



55 Tetraethoxyethyl-bis-pyridinium perchlorate

(II)



p-t-Octylphenoxypropylpolyethoxyethylpyridinium methanesulfonate (a derivative of an ethylene oxide and p-tert-octylphenol in which  $n$  has an average value of 4.)

(III)



Octaethoxyethyl-bis-pyridinium perchlorate

(IV)



Octaethoxyethyl-bis-trimethylammonium perchlorate

(V)



Octaethoxyethyl-bis-dimethyldecylammonium perchlorate

(VI)



Tetraethoxyethyl-bis-dimethylsulfonium perchlorate

(VII)



p-t-Octylphenoxypropylpolyethoxyethyldimethylsulfonium-p-toluene sulfonate (in which  $n$  has an average value of 4)

(VIII)



Polyethoxyethyl-bis-pyridinium perchlorate (in which the polyethyleneoxy chain is derived from a polyethylene glycol having a molecular weight of about 300).

The quaternized polyalkylene oxide monoethers having formulas B and E above are prepared by reaction of the appropriate polyalkylene oxide monoethers such as



or methoxypolyethylene oxide, with alkylsulfonyl halides such as methanesulfonyl chloride, ethanesulfonyl chloride, p-toluenesulfonyl chloride, followed by quaternization with tertiary bases as pyridine, picolines and trialkylamines such as trimethylamine, dimethylbenzylamine, dimethyllaurylamine, etc. The resulting quaternary salts may be converted to salts of other anions such as the perchlorate in order to facilitate purification.

The bis-quaternary compounds of formulas A and D above are prepared by reaction of polyalkylene oxides of varying molecular weight, with the just above sulfonyl halides, followed by quaternization as described just above. Thus, polyalkylene oxides such as polyethylene oxides having average molecular weights of the order of about 200 to 1500 or more can be employed to provide the polyalkylene oxide radical of the sensitizers.

The cationic quaternary and ternary polyalkylene oxide sensitizers can be used in the emulsion with useful results in concentrations of the order of from about 0.1 gram to 6.0 grams per mole of silver halide present in the emulsion.

The syntheses of the following cationic materials also useful in the emulsions are described in the co-filed invention of Carroll, Sagal and Beavers U.S. patent application Serial No. 627,135.

3,6,9,12,15,18,21,24 - octoxahexacosane - 1,26 - bis(pyridinium methanesulfonate)

3,6,9,12,15,18,21,24 - octoxahexacosane - 1,26 - bis(pyridinium perchlorate)

3,6,9,12,15,18,21,24 - octoxahexacosane - 1,26 - bis(trimethylammonium perchlorate) (Compound IV)

Polypropoxypropyl- $\alpha$ - $\omega$ -bis - (pyridinium methanesulfonate)-containing about 16 isopropoxy units

Polypropoxypropyl- $\alpha$ - $\omega$ -bis - (pyridinium methanesulfonate)-containing about 6 isopropoxy units

5

The anionic polyalkylene oxide sensitizers are of various types including, e.g., the polyalkylene oxide carboglutamic acid salts, N-carboxymethyl carbamate salts and polyalkylene oxide sulfuric acids. These anionic materials are characterized by containing at least 4 and preferably at least 13 bivalent polyalkylene oxide radicals, such as polyethylene oxide, polypropylene oxide and polybutylene oxide radicals, to which is attached at least one anionic group. The following are representative anionic polyalkylene oxide sensitizers useful in our invention.

10



20



30



35



40



45



50



55



60



65



70



75

The above anionic polyalkylene oxide compounds are prepared as illustrated below:

COMPOUND XII (*n*=8)

*Nonaethylene glycol- $\alpha,\omega$ -disulfonic acid, disodium salt  
nonaethylene glycol- $\alpha,\omega$ -dichloride*

Nonaethylene glycol, 103.5 g. (0.25 mole), was dissolved in 40 g. (0.50 mole) of dry pyridine, and the solution chilled to 0° C. With rapid stirring, 59.0 g. (0.50 mole) of thionyl chloride was slowly added maintaining the temperature at 0–10°. During the addition a thick slurry formed. The slurry was allowed to stand overnight at room temperature, poured into 400 ml. of ice water, and the product extracted three times with 250 ml. portions of benzene. The extracts were dried over sodium sulfate, and the solvent removed leaving 65.0 g. of a dark yellow oil. The oil was fractionated, the desired portion being collected at 237–243°/0.1–0.2 mm. and weighing 26.0 g. (23 percent yield).

*Analysis.*—Calc. for  $C_{18}H_{36}O_8Cl_2$ : Cl, 16.0. Found: Cl, 16.0.

Nine grams (0.02 mole) of nonaethylene glycol-dichloride was dissolved in 175 ml. of ethanol, and this solution was added to 4.9 g. (0.04 mole) of sodium sulfite in 100 ml. of water. The mixture was refluxed for eighteen hours with vigorous stirring. The aqueous ethanol was removed leaving a waxy solid. The wax was dissolved in 100 ml. of hot absolute ethanol, and the inorganic salt filtered off. The filtrate was concentrated to dryness giving a waxy cream colored solid weighing 8.5 g. (73 percent). The absence of chloride ion was demonstrated with a solution of silver nitrate.

COMPOUND XII (*n*=35)

Polyethylene oxide molecular weight 1540, 144 g. (0.093 mole) was dissolved in 400 ml. of dichloromethane. The clear solution was cooled to 0° C., and a steady stream of nitrogen bubbled through a sintered glass tip under the surface of the liquid while 21.6 g. (0.185 mole) of chlorosulfonic acid was slowly added. The solution was maintained at 0° for 2 hours while the rapid stream of nitrogen drove out the hydrogen chloride formed in the reaction. The solution was allowed to stand overnight, and the dichloromethane removed under vacuum to 45°. Upon cooling, 156 g. (97 percent) of an amber liquid solidified to a waxy cream solid. The bisulfuric acid darkened slowly upon standing and rapidly upon heating. An aqueous solution of the bisulfuric acid showed no presence of chloride ion with a silver nitrate solution.

COMPOUND XII (*n*=75)

To 200 ml. of dichloromethane, 33.5 (0.01 mole) of polyethylene oxide (average molecular weight 3000–3700) was added and the solution cooled to 0° C. With a vigorous stream of nitrogen passed into the mixture, 2.33 g. (0.02 mole) of chlorosulfonic acid was added with stirring. After two hours at 0° in the nitrogen stream, the solution was allowed to warm up to room temperature and the dichloromethane removed under vacuum to 45° C. The product was a light amber oil weighing 31.0 g. (88.5 percent) which solidified to a white wax upon cooling.

COMPOUND XIX

One hundred and four grams (0.14 mole) of



was dissolved in 400 ml. of dichloromethane and the solution cooled to 0°. Then 16.0 g. (0.14 mole) of chlorosulfonic acid was added, with a rapid stream of nitrogen bubbled through the solution which removed the hydrogen chloride formed. The solution was stirred at 10° for three hours in the stream of nitrogen. The dichloromethane was removed under vacuum at 40°, leaving 115.0 g. of a brown, viscous syrup (99 percent yield).

COMPOUND XIII

A mixture of 137 g. of polyethylene oxide molecular weight 1540 and 36 g. of dimethyl isocyanatoglutarate was heated at 70°±5° for twenty-four hours. During the heating the mixture was protected from atmospheric moisture. The product was transferred to a beaker and selectively hydrolyzed by treatment with four molar equivalents (14.5 g.) of sodium hydroxide in 35 ml. of water. The alkaline solution was added in portions with stirring, while the temperature was maintained at 60–70°. The mixture was then heated for 3 hours at 60–70°, water being added occasionally so as to maintain the material in a fluid state. It was diluted with water to give a 48 percent solution which was filtered.

15

COMPOUND XI

The product resulting from heating 80 g. of polyethylene oxide molecular weight 4000 with 6 g. of ethyl isocyanatoacetate for 4 hours on the steam bath while protected from atmospheric moisture was treated with 1.6 g. of sodium hydroxide dissolved in about 5 ml. of water. Heating was continued on the steam bath for two hours, during which time additional amounts of water were added to maintain the product in a fluid state. Water was added to give a total weight of 150 g. Such a solution contains an estimated 85 g. (57 percent) of solids.

25

COMPOUND XVI

The product obtained by heating together 87 g. of the oleyl ether of polyethylene glycol molecular weight 525 and 22 g. of dimethyl isocyanatoglutarate at 60–70° for 20 hours in the absence of atmospheric moisture was treated with 9 g. of sodium hydroxide in 25 ml. of water. The mixture was heated for two hours at 60–70°, water being added in small quantities to maintain the mixture in a fluid state. It was finally diluted with water to yield a 42 percent aqueous solution (111 g. of solid in a total weight of 262 g.) of a product that is essentially

30



in which *n* has the average value of 12.

35

COMPOUNDS XVII and XVIII

In a similar manner the cetyl ether of polyethylene glycol and dimethyl isocyanatoglutarate gave N-carbobetylxyloxyethoxy-ethyl-glutamic acid (sodium salt), and the p-tert-octylphenyl ether of polyethylene glycol and dimethyl isocyanatoglutarate gave N-carbo-p-tert-octylphenoxyethoxyglutamic acid (sodium salt). In the former case the molecule contained an average of 27  $CH_2CH_2O$  units; in the latter an average of 30 units.

40

COMPOUND X

The amine



45

was dissolved in absolute acetone and one equivalent of the acid chloride  $CH_3COO(C_2H_4O)_{34}CH_2COCl$  was added to the solution at room temperature. After stirring 10 min. one equivalent of quinoline was added and the reaction mixture was refluxed with stirring for 1.5 hours.

50

The reaction mixture was cooled, the quinoline hydrochloride precipitate was filtered out and the acetone removed under reduced pressure. The residue was crystallized from 60–40 benzene-ligroin (B.P. 100–110° C.). The product white needles, had an M.P. of 49–50° C.

The amine is described in McCrossen et al. U.S. Patent 2,688,544, September 7, 1954.

The acid chloride was prepared by treating an excess of the polyglycol with metallic sodium, reacting the sodium salt with chloroacetic acid followed in turn by acetic anhydride and thionyl chloride.

ANALYSIS OF COMPOUND X

|         | Calcd. for<br>$C_{102}H_{170}Cl_2N_2O_{40}$<br>percent | Found,<br>percent |
|---------|--------------------------------------------------------|-------------------|
| C.....  | 57.5                                                   | 56.7              |
| H.....  | 8.2                                                    | 8.5               |
| Cl..... | 3.3                                                    | 3.4               |
| N.....  | 1.3                                                    | 1.5               |

COMPOUND II

To a solution of 42.6 g. (0.1 mole) of p-tert-octylphenoxytetraethoxyethanol and 11 g. (0.109 mole) of triethylamine (anhydrous) in dry ethyl ether chilled to 0° C. is added, in portions, 11.5 g. (0.1 mole) of methanesulfonyl chloride. The mixture is shaken thoroughly and allowed to stand at room temperature for 3 days. The triethylamine hydrochloride that separates is removed by filtration. Removal of the ether leaves 50 g. of a clear, colorless liquid.

A mixture of 5.03 g. (0.01 mole) of the above liquid and 0.8 g. (0.01 mole) of pyridine is heated on the steam bath for 18 hours. The resulting liquid which is quite soluble in water is essentially p-tert-octylphenoxytetraethoxyethylpyridinium methanesulfonate.

Compounds which are most efficacious for use in the emulsions together with the ionic polyalkylene oxide compounds for reducing fog to normal levels are the azaindenes, for example, a 4-hydroxy-6-alkyl-1,3,3a,7-tetraazaindene specifically 4-hydroxy-6-methyl-1,3,3a,7-tetraazaindene as well as 5-carboxy-4-hydroxy-1,3,3a,7-tetraazaindene, (Reynolds U.S. Application Serial No. 520,120, filed July 5, 1955), 1,2-bis(4-hydroxy-6-methyl-1,3,3a,7-tetraazaindene-5-yl)ethane, 1,2,3,4-tetrakis(4-hydroxy-6-methyl-1,3,3a,7-tetraazaindene-2-yl)butane, 2-amino-5-carboxy-4-hydroxy-1,3,3a,7-tetraazaindene, 4-hydroxy-2-β-hydroxyethyl-6-methyl-1,3,3a,7-tetraazaindene, 5-carbethoxy-4-hydroxy-1,3,3a,7-tetraazaindene, (Reynolds invention above), 7-hydroxy-1,2,3,4,6-pentazaindene, 2,4-dihydroxy-6-methyl-1,3a,7-tetraazaindene, 4-hydroxy-2-γ-hydroxypropyl-6-methyl-1,3,3a,7-tetraazaindene and 4-hydroxy-2-(4-pyridyl)-6-methyl-1,3,3a,7-tetraazaindene.

Other azaindene compounds useful for this purpose are disclosed in the examples hereinafter, in U.S. Patents 2,716,062, 2,713,541 and

U.S. Patent 2,735,769, Allen et al., issued February 21, 1956,

U.S. Patent 2,743,181, Allen et al., issued April 24, 1956, U.S. application S.N. 515,785, Tinker et al., filed June 15, 1955,

U.S. Patent 2,756,147, Reynolds, issued July 24, 1956, U.S. Patent 2,743,180, Carroll et al., issued April 24, 1956,

Zeitschrift fur Wiss. Phot. 47, 2-28 (1952).

However, the speed increases are nevertheless obtained using the ionic polyalkylene oxide compounds in the absence of such antifoggants as attested by the examples hereinafter

4-hydroxy-6-methyl-1,3,3a,7-tetraazaindene can be prepared as follows:

A mixture of 108.8 kg. (800 moles) aminoguanidine bicarbonate and 44.8 kg. (877 moles) formic acid (90%) was refluxed overnight in a 100-gal. jacketed, glass-lined kettle. The steam pressure was set at 25 p.s.i. In the morning the reaction mixture was diluted with 601 hot water and 10.4 kg. (98 moles) anhydrous sodium carbonate was added slowly. The run was heated for three hours at 90-100° and was then concentrated under vacu-

um until no more water distills over (about 4-5 hr.). The residue was a mushy, white solid which was cooled overnight under vacuum. Then, 144 kg. glacial acetic acid and 150 kg. (1150 moles) ethyl acetoacetate were added and the mixture is refluxed for three hours. The run was cooled to room temperature and dropped into a 150-gal. stainless steel tank. The liquors were removed by filtration and saved for recovery. The solid was slurried in 30 gal. alcohol, filtered and centrifuged.

10 Washing with fresh portions of alcohol was repeated until no additional color is removed and the odor of acetic acid was at a minimum. The white to pale pink needles were dried on paper trays in a warm air oven. The melting point is 285-287°. The yield was 98 kg.

15 This is 81.5% of the theoretical quantity—120 kg.

7-hydroxy-1,2,3,4,6-pentazaindene

A solution of 50 g. (0.22 moles) of 4,5-diamino-3-hydroxypyrimidine sulfate, J. Am. Chem. Soc. 74, 411 (1952) and 18 g. of sodium nitrite in 300 ml. of 10 percent sodium hydroxide solution was slowly acidified by the addition of acetic acid. The mixture was stirred on the steam bath for 30 minutes and cooled overnight in the refrigerator. The solid was collected on a Buchner funnel and recrystallized from 5 percent hydrochloric acid and then from water to give 30 g. (99%) of the product.

Analysis.—Calcd. for  $C_4H_3N_5O$ : C=35.0; H=2.7. Found: C=35.0; H=2.7.

2,4-dihydroxy-6-methyl-1,3a,7-triazaindene

To a solution of 18.4 g. (0.8 moles) of sodium in 500 ml. of dry methanol was added 23.4 g. (0.2 moles) of guanidoacetic acid followed by 52 g. (0.4 moles) of ethyl acetoacetate. The mixture was refluxed for 20 hours, concentrated, washed with ether, and taken up in 5 percent hydrochloric acid until the solution had a pH 1 (about 600 ml. of acid). The insoluble material was collected and recrystallized from water to give 5 g. of product melting at 310° C.

1,2-bis-4-hydroxy-6-methyl-1,3,3a,7-tetraazaindene-5-yl ethane

A mixture of ethyl  $\alpha,\alpha'$ -diacetylalipate (29 g.) (H518-20) and 3-amino-1,2,4-triazole (17 g.) in 100 ml. of acetic acid was refluxed 4 hours, cooled, and the solid collected. The solid was digested with 800 ml. of boiling dimethylformamide, filtered hot, and washed with ethanol to yield 20 g. (plus 2 g. from the filtrate) of product melting above 310 degrees.

Analysis.—Calcd. for  $C_{14}H_{14}N_8O_2$ , C=51.5, H=4.3, N=34.4. Found: C=51.5, H=4.7, N=34.5.

2-amino-5-carboxy-4-hydroxy-1,3,3a,7-tetraazaindene

A mixture of guanazole (25 g.) and diethyl ethoxy-methylene malonate (56 g.) in 150 ml. of acetic acid was refluxed 4 hours, cooled and the 2-amino-5-carboxy-4-hydroxy-1,3,3a,7-tetraazaindene collected on a Büchner funnel and dried (46.5 g., 83%).

60 The ester (25 g.) and 250 ml. of 1 N hydrochloric acid were refluxed 4 hours, cooled, and the solid collected and recrystallized from water to give 9 g. of the acid (M.P. above 300° C.).

Analysis.—Calcd. for  $C_6H_5N_5O_3$ : C=37, H=2.5, N=35.9. Found: C=37.9, H=2.8, N=35.6.

4-hydroxy-2-β-hydroxypropiohydrazido-6-methyl-pyrimidine

A mixture of 246 grams of  $\beta$ -hydroxypropiohydrazide (267 moles, 50% excess) (J.A.C.S., 73, 3168), 300 grams of 2-ethylmercapto-4-hydroxy-6-methyl-pyrimidine (1.77 moles) (Ber., 86, 1403), 1 liter of ethanol and 1 liter of water was refluxed 18 hours. Precipitation begins after about 15 hours, continued refluxing for 24 hours longer (total 42 hours). Cooled to 25°, filters

212 grams, 57%, M.P. 223-226°. Recrystallization from water raises the M.P. to 233-234°.

4-hydroxy-2-β-hydroxyethyl-6-methyl-1,3,3a,7-tetrazaindene

Sixty-three grams of hydrazide was refluxed 20 hours in 500 ml of glacial acetic acid and 50 ml. of concentrated hydrochloric acid. The hot solution was filtered, then cooled, yielding 12 grams of white solid, M.P. 257-260°. A second recrystallization from water yielded 6.5 grams (10%) of pure anhydrous material, M.P. 262-263°.

*Analysis.*—Calcd.: C, 49.4; H, 5.2; N, 28.9 ( $C_8H_{10}N_4O_2$ , 194). Found: C, 49.7; H, 4.9; N, 27.2.

1,2,3,4-tetrakis(4-hydroxy-6-methyl-1,3,3a,7-tetrazaindene-2-yl)butane

One hundred ninety-five grams of 1,2,3,4-tetrakis(carbohydrazido)butane (formed by reacting 1,2,3,4-tetracarbomethoxybutane with hydrazine), 340 grams of 2-ethyl-mercapto-4-hydroxy-6-methylpyrimidine, 100 ml. of glacial acetic acid and 5 liters of water refluxed 24 hours, cooled well, and filtered.

This crude 1,2,3,4-tetrakis(4-hydroxy-6-methyl-2-pyrimidylhydrazino)butane was refluxed with 1 liter of glacial acetic acid, and 50 ml. of concentrated hydrochloric acid for 24 hours, cooled to 0°, and filtered. The solid, recrystallized from water, yielded 39 grams of 6-methyluracil, M.P. 310-315° (infrared spectrum, 6143A identical with that of an authentic sample, 6096A). The combined mother liquors evaporated and recrystallized from water, eventually yielded 18 grams of white solid, M.P. 263-265°; the infrared spectrum of which is different from that of 6-methyluracil and of 2,6-dimethyl-4-hydroxy-1,3,3a,7-tetrazaindene. The analytical figures agree fairly well with the tetrahydrate, but suggest slightly incomplete conversion of carboxyl to tetrazaindene moieties.

*Analysis.*—Calcd: C, 46.5; H, 4.7; N, 31.0



Found: C, 48.9; H, 5.0; N, 27.5.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, *The Theory of the Photographic Process*, 1942, page 3). The sensitizing agents may be added at any stage, preferably after the final digestion.

The photographic emulsions which we use are of the developing-out type and best results have been obtained with gelatino-silver bromoiodide emulsions. However, emulsions of varying silver halide content may be used.

The emulsions may be chemically sensitized by any of the accepted procedures, in addition to sensitizing with the ionic polyalkylene oxide compounds. The emulsions may be digested with naturally active gelatin, or sulfur compounds may be added such as those described in Sheppard U.S. Patents 1,574,944 and 1,623,499, and Sheppard and Brigham U.S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladate, which are used for sensitizing in amounts below that which produces any substantial fog inhibition, as described in Smith and Trivelli U.S. Patent 2,448,060, and as antifoggants in higher amounts, as described in Trivelli and Smith U.S. Patents 2,566,245 and 2,566,263.

The emulsions may also be chemically sensitized with

gold salts as described in Waller and Dodd U.S. Patent 2,399,083 or stabilized with gold salts as described in Damschroder U.S. Patent 2,597,856 and Yutzy and Leermakers U.S. Patent 2,597,915. Suitable compounds are potassium chloroaurite, potassium aurithiocyanate, potassium chloroaurate, auric trichloride and 2-aurosulfobenzothiazole methochloride.

The emulsions may also be chemically sensitized with reducing agents such as stannous salts (Carroll U.S. Patent 2,487,850), polyamines such as diethylene triamine (Lowe and Jones U.S. Patent 2,518,698), polyamines such as spermine (Lowe and Allen U.S. Patent 2,521,925), or bis-(β-aminoethyl) sulfide and its water-soluble salts (Lowe and Jones U.S. Patent 2,521,926).

As mentioned, when using the ionic polyalkylene oxide derivatives for sensitizing the emulsions, any undesirable fog can be suppressed and reduced to normal levels by using various compounds such as the mercury compounds of Allen, Byers and Murray U.S. Patent 2,728,663, Carroll and Murray U.S. Patent 2,728,664, and Leubner and Murray U.S. Patent 2,728,665 granted December 27, 1955, and the organic mercury compounds of the parent invention of which this application is a continuation-in-part.

Other stabilizing agents may be added to the emulsions containing the polyalkylene oxide salts such as cadmium chloride, cadmium nitrate, cobalt nitrate, manganese chloride, manganese sulfate, zinc chloride, zinc nitrate and zinc sulfate.

The chemical sensitizing agents and other addenda which we have described may be used in various kinds of photographic emulsions, e.g. various silver salts may be used as the sensitive salt such as silver bromide, silver iodide, silver chloride or mixed silver halides such as silver chlorobromide or silver bromoiodide.

The dispersing agent for the silver halide may be gelatin or other hydrophilic material such as collodion, albumin, cellulose derivatives or synthetic resins.

Since the coupler-containing emulsions sensitized as described with the ionic polyalkylene oxide salts are adapted particularly for use in color photography, they will ordinarily comprise the emulsion layers of multilayer color films which emulsion layers are customarily differentially sensitized to the primary regions of the visible spectrum and contain coupler compounds producing dye images of colors complementary to the sensitivity of the emulsion layers. In a representative color film, one or more of the differentially sensitized emulsion layers may be sensitized with the ionic polyalkylene oxide salts, and in a typical example emulsions sensitized to the red, green and blue regions of the spectrum are superimposed on the support in that order and contain cyan, magenta and yellow color-forming coupler compounds respectively. A yellow filter layer such as yellow colloidal silver is advantageously interposed between the blue and green-sensitive emulsion layers.

Since the emulsion layers sensitized with the ionic polyalkylene oxide salts of the invention contain coupler compounds they can be readily processed by well known methods to yield color negatives directly or positive images by means of well known reversal processes. That is, after initial exposure of the emulsion to a subject a developer of the p-phenylenediamine type will produce a colored image negative in respect to the subject. Likewise, if development of the emulsion layer is first carried out with a non-color-forming developer followed by reversal exposure of the residual silver halide and then color development, a colored positive is obtained.

The coupler compounds used in the emulsion layers sensitized with the ionic polyalkylene oxide derivatives, are any of the well known compounds which combine with the oxidation product of primary aromatic amino silver halide color developing agents to form dyes, for example, the phenolic couplers of U.S. Patents 2,266,452, 2,362,598, 2,589,004, 2,474,293, 2,521,908, 2,423,730 and

Fierke U.S. Patent application 476,561; the pyrazolone couplers of U.S. Patents 1,969,479, 2,369,489, 2,600,788, 2,618,641, 2,511,231 and the open chain reactive methylene couplers of U.S. Patents 2,298,443, 2,652,329, 2,407,210, 2,271,238 and McCrossen et al. U.S. Patent Application Serial No. 575,099, filed March 30, 1956. Likewise, the emulsions may contain colored color-forming couplers as described in U.S. Patents 2,521,908, 2,706,684, 2,455,169, 2,694,703, 2,455,170 and 2,453,661.

The couplers may be dispersed in the emulsion layers by means of an oily coupler solvent according to the methods of U.S. Patents 2,304,940 and 2,322,027. However, if as may be the case, the couplers contain solubilizing groups such as  $\text{SO}_3\text{H}$  groups which render the couplers soluble in alkaline solution, the oily coupler solvent may be dispensed with and the couplers can be added to the emulsion from aqueous solutions as their alkali metal salts.

The following examples will serve to illustrate our invention:

*Example 1.*—This example illustrates a known chemical sensitizing effect of unquaternized polyalkylene oxides.

A negative speed gelatino-silver bromoiodide emulsion adjusted to optimum sensitivity with a mixture of a labile sulfur compound and a soluble gold salt was divided into two portions. To each portion was added, at 40° C., an equal amount of an optical sensitizing dye that sensitized the emulsion in the region 5000–6000 Å. Each portion was then treated, before coating on a suitable support, as indicated below.

(a) Control—no further treatment.

(b) 1.69 g. per mole of silver halide of the oleyl ether of a polyethylene oxide of molecular weight of about 1500, was added before coating. The resulting coatings were tested sensitometrically by exposure from  $\frac{1}{50}$ " through a green filter to studio quality light on an intensity scale sensitometer (Eastman Ib) and developed 10 minutes at 75° F., with intermittent agitation in an Elon-hydroquinone developer. The following results were obtained:

| Sample   | Speed <sup>1</sup> | Min. Density |
|----------|--------------------|--------------|
| (a)..... | Control.....       | .06          |
| (b)..... | +10.....           | .09          |

<sup>1</sup> Speed is expressed as 100 (1-log E) where "E" is the exposure in meter candle seconds required to produce in the processed film a silver density of 0.20 above minimum density.

A similar effect is obtained when the development is carried out with a p-phenylenediamine type of developer.

The developer used above had the same composition as the negative developer shown in Example 2 hereinafter.

*Example 2.*—This example illustrates the mentioned effect of sensitizing a coupler-containing emulsion with a non-ionic polyalkylene oxide.

A negative-speed gelatino-silver bromoiodide emulsion adjusted to optimum sensitivity with a mixture of a labile sulfur compound and a soluble gold salt was divided into two portions. To each portion was added, at 40° C., an equal amount of an optical sensitizing dye that sensitized the emulsion in the region 5000–6000 Å and equal amounts of a magenta-forming color coupler of the pyrazolone type, 1-(2,4,6-trichlorophenyl)-3,3'-(2",4"-di-t-amylphenoxy-acetamido)-benzamido-1,5-pyrazolone, suitably dispersed in a high-boiling lyophobic solvent. Each portion was then treated before coating on a suitable support as indicated below.

(a) Control—no further treatment.

(b) 1.69 g./silver mole of the above oleyl ether of polyethylene oxide was added before coating. The resulting coatings were tested sensitometrically by exposing in the same manner as the coatings in Example 1, devel-

oping to a color positive using the following commercial color process carried out at 75° F.:

|                             | Minutes |
|-----------------------------|---------|
| (1) Negative development    | 10      |
| (2) Reversal flash exposure | —       |
| (3) Color development       | 15      |
| (4) Silver bleaching        | 8       |
| (5) Fixing                  | 3       |

The negative developer had the following composition:

|                                              |       |      |
|----------------------------------------------|-------|------|
| Water, 90° F. (32° C.)                       | liter | 1.0  |
| Sodium hexametaphosphate                     | grams | 2.0  |
| N-methyl p-aminophenol sulfate               | do    | 6.0  |
| Sodium sulfite, desiccated                   | do    | 50.0 |
| 15 Hydroquinone                              | do    | 6.0  |
| Sodium carbonate, monohydrated               | do    | 35.0 |
| Potassium bromide                            | do    | 2.0  |
| Sodium thiocyanate                           | do    | 1.5  |
| 0.5% Solution (6-nitrobenzimidazole nitrate) | cc    | 12.0 |
| 20 0.1% Solution of potassium iodide         | cc    | 10.0 |

The color developing solution above had the following composition:

|                                                                                              |       |       |
|----------------------------------------------------------------------------------------------|-------|-------|
| Water, 70° to 80° F. (21° to 27° C.)                                                         | liter | 1.0   |
| Benzyl alcohol                                                                               | cc    | 6.0   |
| Sodium hexametaphosphate                                                                     | grams | 2.0   |
| Sodium sulfite, desiccated                                                                   | do    | 5.0   |
| 30 Trisodium phosphate                                                                       | do    | 40.0  |
| Potassium bromide                                                                            | gram  | 0.25  |
| 0.1% Solution of potassium iodide                                                            | cc    | 10.0  |
| Sodium hydroxide                                                                             | grams | 6.0   |
| 4-amino-N-ethyl-N-[ $\beta$ -methane-sulfonamido-ethyl]m-toluidine sesquisulfate monohydrate | grams | 11.33 |
| Ethylenediamine sulfate                                                                      | do    | 7.8   |
| 35 Citrazinic acid (2,6-dihydroxyiso-nicotinic acid)                                         | grams | 1.5   |

The silver bleaching solution above had the following composition:

|                           |       |      |
|---------------------------|-------|------|
| 40 Water, 90° F. (32° C.) | liter | 1.0  |
| Potassium dichromate      | grams | 5.0  |
| Potassium ferricyanide    | do    | 70.0 |
| Potassium bromide         | do    | 20.0 |

45 The fixing baths above had the following composition:

|                        |       |       |
|------------------------|-------|-------|
| Water, 80° F. (27° C.) | liter | 1.0   |
| Sodium thiosulfate     | grams | 150.0 |
| Sodium bisulfite       | do    | 20.0  |

50 The following results were obtained:

| Sample   | Speed <sup>1</sup> | Max. Density |
|----------|--------------------|--------------|
| (a)..... | Control.....       | Control.     |
| (b)..... | +4.....            | +10.         |

<sup>1</sup> "Speed" is expressed as 100 (1-log E) where E is the exposure in meter candle seconds required to produce after processing a total dye density of 1.0 to appropriate illumination.

60 In the above data of the table, it will be apparent that sample "b" has higher maximum density than "a" since the lower sensitivity of "b" resulted in less silver halide being developed in the negative development step.

*Example 3.*—The improvement in emulsion speed obtained by sensitizing emulsions containing couplers with the cationic polyalkylene oxide salts according to our invention is illustrated in this example.

A negative-speed gelatino-silver bromoiodide emulsion adjusted to optimum sensitivity with a mixture of a labile sulfur compound and a soluble gold salt was divided into three portions. To each portion was added, at 40° C., an equal amount of an optical sensitizing dye that sensitized the emulsion in the region 5000–6000 Å and equal amounts of a magenta-forming color coupler of the pyrazolone type (Example 2) suitably dispersed in a high-

boiling lyophobic solvent. Each portion was then treated, before coating on a suitable support, as indicated below.

(a) Control—no further treatment.

(b) 2 g. per mole of silver halide of polyethoxyethyl-bis-pyridinium perchlorate (compound VIII above, the carbon chain of which has a molecular weight of about 1500), was added before coating.

(c) 2 grams per mole of silver halide of tetraethoxyethyl-bis-pyridinium perchlorate (compound I above) was added before coating. The resulting coatings were tested sensitometrically by exposing and processing to a color positive in the same manner as the coatings in Example 2. The following results were obtained:

| Sample | Speed <sup>1</sup> | Max. Density |
|--------|--------------------|--------------|
| (a)    | Control            | Control      |
| (b)    | +10                | .04          |
| (c)    | +16                | .16          |

<sup>1</sup> "Speed" is determined in the manner indicated in Example 2.

The increased speed of samples *b* and *c* clearly show the effectiveness of the polyalkylene oxide salt sensitizing agents of the invention when used in combination with the coupler compound.

*Example 4.*—A negative-speed gelatino-silver bromoiodide emulsion digested to optimum sensitivity with a mixture of labile sulfur compound and a soluble gold salt was divided into two portions. To each portion was added, at 40° C., an equal amount of an optical sensitizing dye that sensitized the emulsion in the region 5000-6000 Å and equal amounts of a magenta-forming color coupler of the pyrazolone type, suitably dispersed in a high-boiling lyophobic solvent. Each portion was then treated, before coating on a suitable support, as indicated below.

(a) Control—no further treatment.

(b) 2.0 g. per mole of silver halide of compound III above was added before coating.

The resulting coatings were tested sensitometrically by exposing for  $\frac{1}{60}$ " through a yellow filter to light of studio light (3150° K.) quality on an intensity scale sensitometer (Eastman Ib) and developed to a color negative in Developer SD-30 (described in the Journal of the Society of Motion-Picture and Television Engineers, vol. 61, No. 6, p. 674, December 1953). The following results were obtained:

| Sample | Speed <sup>1</sup> | Minimum Density |
|--------|--------------------|-----------------|
| (a)    | 215                | 0.27            |
| (b)    | 254                | 0.44            |

<sup>1</sup> "Speed" is expressed as 100 (1-log E) where "E" is the exposure in meter-candle-seconds required to produce in the processed film a magenta dye density to green light of 0.20 above minimum green light density.

In the table, the comparatively higher "minimum density" value of 0.44 reflects the mentioned desirability of using an antifoggant in the emulsions sensitized with the polyalkylene oxide salts to reduce fog.

*Example 5.*—A negative-speed gelatino-silver bromoiodide emulsion digested to optimum sensitivity with a mixture of labile sulfur compound and a soluble gold salt was divided into two portions. To each portion was added, at 40° C., an equal amount of an optical sensitizing dye that sensitized the emulsion in the region 5000-6000 Å and equal amounts of a magenta-forming color coupler of the pyrazolone type (Example 2), suitably dispersed in a high-boiling lyophobic solvent. Each portion was further treated, before coating on a suitable support, as described below:

(c) Control—no further treatment.

(d) 2.0 g. per mole of silver halide of compound III above was added.

The resulting coatings were exposed for  $\frac{1}{60}$ " to the

light emitted by a 500 w. tungsten lamp in an intensity scale sensitometer, further modulated by a green filter and a 0.6 neutral density filter. The exposed coatings were processed as follows:

(1) Developed for 10' at 75° F. with intermittent agitation, in the negative developer of Example 2.

(2) Fixed 5' in acid-hypo fixing solution.

(3) Washed 10' in running water.

(4) Rehalogenized for 10' in a bath composed of 70 g. 10 potassium ferricyanide and 20 g. potassium bromide/liter of distilled water.

(5) Washed 10' in running water.

(6) Processed to a color negative as described for the coatings in Example 4.

15 The following results were obtained:

| Sample | Speed <sup>1</sup> | Minimum Density |
|--------|--------------------|-----------------|
| (c)    | Control            | .07             |
| (d)    | +24                | .27             |

<sup>1</sup> "Speed" determined as in Example 4.

As in Example 4, the comparatively high minimum density value of .27 indicates the desirability of using an antifoggant in the emulsion.

*Example 6.*—A negative-speed gelatino-silver bromoiodide emulsion was digested to optimum sensitivity with a mixture of labile sulfur compound and a soluble gold salt and treated with an optical sensitizing dye that sensitized in the region of 6000-7000 Å. At 40° C. there was added a cyan color-forming coupler (6-[ $\alpha$ -(4-[ $\alpha$ -(2,4-dichloro-3-methylphenol)-butyramido]phenoxy)acetamido]-2,4-dichloro-3-methylphenol), suitably dispersed in a high-boiling lyophobic solvent. The emulsion was divided into two equal parts and further treated as indicated below.

(e) Control—no further treatment before coating.

(f) 4.0 g. per mole of silver halide of compound III above was added at 40° C. before coating.

The resulting coatings were tested sensitometrically by exposure for  $\frac{1}{60}$ " through a yellow filter to light of daylight quality on an intensity scale sensitometer (Eastman Ib) and developed to a positive in the reversal color process of Example 2. The following results were obtained:

| Sample | Speed <sup>1</sup> | Maximum Density | Minimum Density |
|--------|--------------------|-----------------|-----------------|
| (e)    | reference          | 2.58            | .05             |
| (f)    | +38                | 1.90            | .05             |

<sup>1</sup> "Speed" in the reversal processed coatings is expressed as 100 (1-log E) where "E" is the exposure in meter candle seconds required to produce, after processing, a total dye density to appropriate illumination of 1.0.

55 The comparatively low "maximum density" value of 1.90 above indicates that due to fog, a larger amount of silver halide developed in the negative developer leaves less silver halide for producing the dye image.

60 *Example 7.*—Emulsions were prepared in the manner of Example 6 as follows:

(g) Emulsion like *e* of Example 6 free of antifoggant.

(h) Emulsion like *f* of Example 6 but containing 16.0 g./mole of silver halide of 4-hydroxy-6-methyl-1,3,3a,7-tetraazindene.

65 The following results were obtained after exposure and processing as described in Example 6.

| Sample | Speed <sup>1</sup> | Maximum Density | Minimum Density |
|--------|--------------------|-----------------|-----------------|
| (g)    | Control            | 2.34            | .05             |
| (h)    | +58                | 1.70            | .05             |

<sup>1</sup> "Speed" was evaluated on the same basis as in Example 6.

Example 8.—Emulsions were prepared in the same manner as Example 6 as follows:

(i) Like *e* in Example 6.

(j) Like *f* in Example 6 plus 8.0 g. per mole of silver halide of 4-hydroxy-6-methyl-1,3,3a,7-tetraazaindene and 4.0 g. per mole of silver halide of 1,2-bis (4-hydroxy-6-methyl-1,3,3a,7-tetraazainden-5-yl)-ethane added before coating.

The resulting coatings were exposed and processed like those in Examples 6 and 7. The following results were obtained:

| Sample   | Speed <sup>1</sup> | Maximum Density | Minimum Density |
|----------|--------------------|-----------------|-----------------|
| (i)..... | reference.....     | 2.20            | .07             |
| (j)..... | +58.....           | 1.60            | .07             |

<sup>1</sup> "Speed" values determined as in Example 6.

Coatings (e), (f), (g), (h), (i) and (j) of Examples 6, 7 and 8 were incubated in sealed, foil envelopes for seven days at 120° F. and 50% R.H. After exposure and development as described in Example 6 the following results were obtained:

| Sample     | Speed        | Maximum Density | Minimum Density |
|------------|--------------|-----------------|-----------------|
| 6 (e)..... | Control..... | 2.50            | .05             |
| 6 (f)..... | .....        | 0.20            | .05             |
| 7 (g)..... | Control..... | 2.08            | .06             |
| 7 (h)..... | +60.....     | 1.62            | .05             |
| 8 (i)..... | Control..... | 1.91            | .07             |
| 8 (j)..... | +55.....     | 1.50            | .06             |

The data in the table shows that the pronounced speed increase resulting from the use of the cationic polyalkylene oxide salt sensitizing agents is maintained after storage at elevated temperatures and humidity. No speed values appear in the table for samples 6(e) and 6(f) since neither emulsion contained an antifogging agent and therefore 6(f) developed fairly high fog on incubation and the speed therefore could not be ascertained. However, samples 7(h) and 8(j) containing both the polyalkylene oxide salt sensitizing agent and the azaindene antifogging had speed values of 60 and 55 units greater than the control samples 7(g) and 8(i).

In a similar manner other stabilizing compounds such as the mercury compounds and azaindene compounds mentioned above can be used to lower fog of the sensitized emulsions to normal levels.

Example 9.—A negative-speed gelatino-silver bromoiodide emulsion was digested to optimum sensitivity with a mixture of labile sulfur compound and a soluble gold salt and treated with an optical sensitizing dye that sensitized in the region of 6000-7000 Å. At 40° C. there was added the cyan color former 6-[ $\alpha$ -(4-[ $\alpha$ -(2,4-di-t-amylphenoxy)butyramido]phenoxy)acetamido] - 2,4 - di-chloro-3-methylphenol suitably dispersed in a high boiling lyophobic solvent. The emulsion was divided into several equal parts and further treated before coating as indicated below.

(A) Control—no further treatment.

(B) 4.0 g. per mole of silver halide of polyethoxyethyl- $\gamma$ , $\omega$ -bis-carboglutamic acid, disodium salt (XIII) was added at 40° C. before coating.

(C) 4.0 g. of (XIII) and 4.0 g. of 4-hydroxy-6-methyl-1,3,3a,7-tetraazaindene (AZA) per mole of silver halide were added at 40° C. before coating.

(D) 4.0 g. of polyethoxyethyl- $\gamma$ , $\omega$ -bis-N-carboxymethyl carbamate, disodium salt (XI) per mole of silver halide was added before coating.

(E) 4.0 g. of (XI) and 4.0 g. of (AZA) per mole of silver halide were added before coating.

(F) 4.0 g. of polyethoxyethyl- $\gamma$ , $\omega$ -bisulfuric acid (XII) per mole of silver halide was added before coating.

(G) 4.0 g. of (XII) and 4.0 g. of (AZA) were added before coating.

The resulting coatings were tested sensitometrically by exposure for  $\frac{1}{50}$ " through a red filter to light of daylight quality on an intensity scale sensitometer (Eastman 1b) and developed—

Process A to a silver negative in the first developer of the process of Example 2.

Process B to a reversal color positive in the process of Example 2.

The following results were obtained:

#### PROCESS A

| Sample     | Speed          | Minimum Density |
|------------|----------------|-----------------|
| 15. A..... | Reference..... | Reference.....  |
| B.....     | .....          | .....           |
| C.....     | +12.....       | +.04.....       |
| D.....     | +08.....       | +.06.....       |
| E.....     | +16.....       | +.07.....       |
| F.....     | +04.....       | +.04.....       |
| G.....     | +16.....       | +.04.....       |

#### PROCESS B

| Sample     | Speed          | Maximum Density |
|------------|----------------|-----------------|
| 25. A..... | Reference..... | Reference.....  |
| B.....     | +23.....       | -.28.....       |
| C.....     | +30.....       | -.30.....       |
| D.....     | +35.....       | -.44.....       |
| E.....     | +38.....       | -.50.....       |
| F.....     | +08.....       | -.24.....       |
| G.....     | +26.....       | -.24.....       |

The coatings were incubated in heat-sealed metal foil envelopes for seven days at 120° F./50% R.H. and again tested in Process B. The following results were obtained.

| Sample | Speed          | Maximum Density |
|--------|----------------|-----------------|
| A..... | Reference..... | Reference.....  |
| B..... | +04.....       | -1.08.....      |
| C..... | +40.....       | -.08.....       |
| D..... | -08.....       | -1.72.....      |
| E..... | +51.....       | -.36.....       |
| F..... | +20.....       | -.53.....       |
| G..... | +36.....       | +.17.....       |

The data show the effectiveness of the anionic polyalkylene oxide sensitizers in increasing speed, and in combination with the azaindene compound of maintaining maximum density after incubation.

Example 10.—A negative speed of gelatino-silver bromoiodide emulsion was adjusted to optimum sensitivity with a mixture of labile sulfur compound and a soluble gold salt. At 40° C. there was added the yellow color former N-(4-benzoylacetamidobenzene sulfonyl)-N-( $\gamma$ -phenylpropyl)-p-toluidine suitably dispersed in a high boiling lyophobic solvent. The melt was divided into three equal parts and treated as below:

(a) Control—no further treatment.

(b) 1 g./mole of silver halide of the pyridinium compound III was added at 40° C. before coating.

(c) 1 g./mole of silver halide compound III and 4 g. of 4-hydroxy-6-methyl-1,3,3a,7-tetraazaindene was added at 40° C. before coating.

The resulting coatings were tested sensitometrically in the same manner as Example 4. The following results were obtained:

| Sample   | Speed        | $\Delta$ Minimum Density |
|----------|--------------|--------------------------|
| (a)..... | Control..... | Control.....             |
| (b)..... | +24.....     | +.12.....                |
| (c)..... | +20.....     | +.04.....                |

The coatings were sealed in metal foil envelopes and incubated for 7 days at 120° F./50% R.H. These coatings

were developed to a color negative in the manner described above (Example 4). The following results were obtained:

| Sample   | Speed        | $\Delta$ Minimum Density |
|----------|--------------|--------------------------|
| (a)..... | Control..... | Control.....             |
| (b)..... | -46.....     | +46.....                 |
| (c)..... | +44.....     | -01.....                 |

The values of +44 and -.01 show that the speed is maintained and little fog is obtained upon incubation of the stabilized Sample c.

*Example 11.*—An emulsion melt was prepared as described in Example 6. The melt was divided into three equal parts and further treated as indicated below:

(a) Control—no further treatment.

(b) 4 g./mole of silver halide of compound III above was added before coating.

(c) 4 g./mole of silver halide of compound III and 4 g. per mole of silver halide of 1,2-bis-(4-hydroxy-6-methyl-1,3,3a,7-tetraazaindene-5-yl)-ethane was added before coating. These coatings were exposed and developed to a color positive like those in Example 6. The following results were obtained.

| Sample   | Speed        | $\Delta$ Maximum Density |
|----------|--------------|--------------------------|
| (a)..... | Control..... | Control.....             |
| (b)..... | +15.....     | -.50.....                |
| (c)..... | +23.....     | -.50.....                |

These coatings were incubated for three days at 120° F./50% R.H. and processed in the same manner as the fresh coatings. The following results were obtained.

| Sample   | Speed        | $\Delta$ Maximum Density |
|----------|--------------|--------------------------|
| (a)..... | Control..... | Control.....             |
| (b)..... | +32.....     | -2.10.....               |
| (c)..... | .....        | -1.0.....                |

*Example 12.*—Emulsion melts like that in Example 6 were prepared and divided into several equal parts and further treated as indicated below:

(a) Control—No further treatment.

(b) 2 g./mole of silver halide of p-t-octylphenoxydiethoxyethyl pyridinium methane sulfonate II was added before coating.



(c) Control for (d).

(d) 2 g./mole of silver halide of polypropylene glycol- $\alpha,\omega$ -bis-pyridinium methane sulfonate derived from polypropylene glycol molecular weight 425 was added before coating. These coatings were exposed and developed to a color negative in the manner described in Example 4 and the following results were obtained.

| Sample   | Speed        | $\Delta$ Minimum Density |
|----------|--------------|--------------------------|
| (a)..... | Control..... | Control.....             |
| (b)..... | +8.....      | No change.....           |
| (c)..... | Control..... | Control.....             |
| (d)..... | +16.....     | +32.....                 |

These coatings were also exposed and developed to a color positive in the manner described in Example 6. The following results were obtained.

| Sample   | Speed        | $\Delta$ Maximum Density |
|----------|--------------|--------------------------|
| (a)..... | Control..... | Control.....             |
| (b)..... | -6.....      | -.10.....                |
| (c)..... | Control..... | Control.....             |
| (d)..... | +6.....      | -.20.....                |

*Example 13.*—An emulsion melt like that described in Example 5 was prepared and divided into three equal parts and further treated as follows:

15 (a) Control—no further treatment.

(b) 2 g./mole of silver halide of polyethoxy- $\alpha,\omega$ -bis-pyridinium perchlorate (VIII n=35) was added before coating.

(c) 2 g./mole of silver halide of the bis pyridinium perchlorate I was added before coating.

20 These coatings were tested sensitometrically in the same manner as those in Example 6 and the following results were obtained.

| Sample   | Speed        | $\Delta$ Maximum Density |
|----------|--------------|--------------------------|
| (a)..... | Control..... | Control.....             |
| (b)..... | +10.....     | -.16.....                |
| (c)..... | +16.....     | -.04.....                |

*Example 14.*—The anionic coupler compound X above was added to samples of a coupler-free emulsion prepared as in Example 2 in the amounts shown below. Samples were then processed to a color positive by the method of Example 2 and to a color negative by the process of Example 4 with the following results:

| Gm. X/Mole Ag x | Example 2 Process |                             | Example 4 Process |                             |
|-----------------|-------------------|-----------------------------|-------------------|-----------------------------|
|                 | $\Delta$ D max.   | Speed $\Delta$ Log E Change | $\Delta$ D min.   | Speed $\Delta$ Log E Change |
| 2.....          | -.16              | +15 Log E.....              | 0.02              | +08 Log E.....              |
| 4.....          | -.20              | +18 Log E.....              | 0.02              | +08 Log E.....              |

*Example 15.*—The ionic compounds XI and III were added to coupler-free emulsions prepared as in Example 2 and the following couplers:

50 Coupler I



(U.S. 2,706,685)

Coupler II



70 (U.S. 2,694,718)

with the results shown in the following table after processing in Example 1 process

| Coupler | Polyalkylene Oxide | Gm/mol Ag X | Speed Log E Change | Max. |
|---------|--------------------|-------------|--------------------|------|
| I       | XI                 | 4           | +42                | -30  |
| II      | III                | 2           | +40                | -24  |

Example 16.—Two, three-color reversal films were prepared as follows:

(1) On a suitable-film support were coated successively:

- A red and blue light-sensitive bromoiodide emulsion and a cyan-color former,
- A gelatin interlayer,
- A green and blue light-sensitive bromoiodide emulsion and a magenta-color former,
- A Carey Lea silver-blue light filter layer
- A blue light-sensitive bromoiodide emulsion and a yellow-color former,
- A protective gelatin overcoat.

(2) A multilayer coating like (1) except that to layers (a), (c), and (e) were added before coating 4 g. per mole silver halide of 4-hydroxy-6-methyl-1,3,3a-7-tetrazaindene, and 4 g. per mole silver halide of compound XI.

The coatings were identically exposed and developed to color positives of equal contrasts as described in Example 2 above, with the result that the following sensitivity increases of the latter coating over the former were as follows:

(1) To red light there was a threshold log exposure advantage (expressed as metercandle-seconds) of 0.22.

(2) To green light the threshold log E advantage was 0.12.

(3) To blue light the threshold log E advantage was 0.15.

Example 17.—A three-color reversal film was prepared similar to film 1 of Example 16 except layers (a) and (e) contained 3, 6, 9, 12, 15, 18, 21, 24-octoxahexacosane-bis-pyridinium perchlorate, 4-hydroxy-6-methyl-1,3,3a,7-tetrazaindene and 6-methyl-4-phenyl-mercapto-1,3,3a,7-tetrazaindene. This film was processed as in Example 16 and the following advantages over film 1 of Example 16 which contained no ionic polyalkylene oxide compound were observed.

(1) To red light, a threshold log exposure advantage of 0.34 (log meter candle seconds).

(2) To green light the threshold log E advantage was 0.15.

(3) To blue light the threshold log E advantage was 0.34.

Emulsions chemically sensitized in the manner of the above examples and optically sensitized to the primary regions of the spectrum and further containing coupler compounds for forming subtractively colored dye images on color development may be superimposed on a support to provide multilayer color films which can be processed directly to a negative or indirectly to a color positive using the color processing procedures illustrated in the above examples.

It will be understood that we include within our invention all modifications and equivalents falling within the scope of the appended claims.

We claim:

1. A light-sensitive silver halide emulsion containing a coupler compound capable of reaction with the oxidation product of a primary aromatic amino silver halide developing agent to form a dye, said emulsion containing a sensitizing agent of the class consisting of (1) a water-soluble salt of a compound having the general formula



wherein  $n$  represents a positive integer greater than 3,

10

R represents an alkylene group of from 2 to 4 carbon atoms, X' and Y represent the same radical of the class consisting of

5



15



20



25



wherein  $R_1$ ,  $R_2$  and  $R_3$  each represent alkyl groups, Q represents the non-metallic atoms necessary to complete a pyridyl nucleus, X represents an acid radical, and (2) a compound having said formula wherein X' represents a member of the class consisting of alkoxy and alkylphenoxy groups.

2. The emulsion of claim 1 further containing a hydroxytetrazaindene stabilizing agent.

3. A light-sensitive silver halide emulsion containing (1) a coupler compound capable of reaction with the oxidation product of a primary aromatic amino silver halide developing agent to form a dye, (2) a hydroxytetrazaindene stabilizing agent and (3) a sensitizing agent having the general formula



45

wherein  $n$  represents a positive integer greater than 3, R represents an alkylene group of from 2 to 4 carbon atoms and  $R_1$ ,  $R_2$  and  $R_3$  represent alkyl groups, and X represents an acid radical.

4. A light-sensitive silver halide emulsion containing (1) a coupler compound capable of reaction with the oxidation product of a primary aromatic amino silver halide developing agent to form a dye, (2) a hydroxytetrazaindene stabilizing agent and (3) a sensitizing agent having the general formula



60

wherein  $n$  represents a positive integer greater than 3 and  $R_1$ ,  $R_2$ , and  $R_3$  each represent alkyl groups, X represents an acid radical.

5. A light-sensitive silver halide emulsion containing (1) a coupler compound capable of reaction with the oxidation product of a primary aromatic amino silver halide developing agent to form a dye, (2) a hydroxytetrazaindene stabilizing agent and (3) a sensitizing agent having the general formula



70

wherein  $n$  represents a positive integer greater than 3, R represents an alkylene group of from 2 to 4 carbon atoms,

Q represents the non-metallic atoms necessary to complete a pyridyl nucleus and X represents an acid radical.

6. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a sensitizing agent having the general formula



wherein n represents a positive integer greater than 3, Q represents the non-metallic atoms necessary to complete a pyridyl nucleus and X represents an acid radical.

7. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of a sensitizing agent having the general formula



wherein n represents a positive integer greater than 3, and R represents an alkylene group of from 2 to 4 carbon atoms.

8. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of a sensitizing agent having the general formula



wherein n represents a positive integer greater than 3.

9. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of a sensitizing agent having the general formula



wherein n represents a positive integer greater than 3 and R represents an alkylene group of from 2 to 4 carbon atoms.

10. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of a sensitizing agent having the general formula



11. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a sensitizing agent having the general formula



wherein R represents an alkylphenyl radical, R<sub>1</sub> represents an alkylene group of from 2 to 4 carbon atoms, n represents a positive integer greater than 3, Q represents the non-metallic atoms necessary to complete a pyridyl nucleus and X represents an acid radical.

12. A light-sensitive silver halide emulsion containing (1) a coupler compound capable of reaction with the oxidation product of a primary aromatic amino silver

halide developing agent to form a dye, (2) a hydroxy-tetrazaindene stabilizing agent and (3) a sensitizing agent having the general formula



wherein R represents an alkyl phenyl radical, n represents a positive integer greater than 3, Q represents the non-metallic atoms necessary to complete a pyridyl nucleus and X represents an acid radical.

13. The emulsion of claim 3 wherein the stabilizing agent is 4-hydroxy-6-methyl-1,3,3a,7-tetrazaindene.

14. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a polyethoxyethyl-bis-pyridinium perchlorate, the polyethylene oxide radical of which contains at least 4 ethylene oxide units.

15. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) octaethoxyethyl-bis-pyridinium perchlorate.

16. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) tetraethoxyethyl-bis-pyridinium perchlorate.

17. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of polyethoxyethyl-bis-N-carboxymethyl carbamate.

18. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) a water-soluble salt of polyethoxyethyl-bis-carboglutamic acid.

19. A light-sensitive silver halide emulsion containing (1) a coupler compound capable of reaction with the oxidation product of a primary aromatic amino silver halide developing agent to form a dye, (2) a hydroxy-tetrazaindene stabilizing agent and (3) polyethoxyethyl-bis-sulfuric acid.

20. A light-sensitive silver halide emulsion containing a coupler compound capable of reaction with the oxidation products of a primary aromatic amino silver halide developing agent to form a dye, said emulsion being sensitized with a member of the class consisting of tetraethoxyethyl-bis-pyridinium perchlorate, p-t-octylphenoxypolyethoxyethylpyridinium methane sulfonate, octaethoxyethyl-bis-pyridinium perchlorate, octaethoxyethyl-bis-trimethylammonium perchlorate, octaethoxyethyl-bis-dimethyldecylammonium perchlorate, tetraethoxyethyl-bis-dimethylsulfonium perchlorate, p-t-octylphenoxypolyethoxyethyldimethylsulfonium - p - toluene sulfonate, polyethoxyethyl-bis-pyridinium perchlorate, polyethoxyethyl-bis-N-carboxymethylcarbamate (di-Na salt), polyethoxyethyl-bis-sulfuric acid, polyethoxyethyl-bis-carboglutamic acid (Na salt), N-carbo-lauroxypolyethoxyethylglutamic acid (di-Na salt), polyethoxyethyl-bis(3,5-disulfobenzoate) (tetra Na salt), N-carbooleylloxypolyethoxyethylglutamic acid (di-Na salt), N-carbocetylloxypolyethoxyethylglutamic acid (di-Na salt), N-carbo-p-octylphenoxypolyethoxyethylglu-

23

tamic acid (Na salt) and p-tert-octylphenoxypolyethoxyethylsulfate (Na salt).

## References Cited in the file of this patent

## UNITED STATES PATENTS

2,280,722 Schneider et al. April 21, 1942

5 2,288,226  
2,423,549  
2,436,138  
2,716,062  
2,751,299  
2,757,089

2,784,090

24

|                |               |
|----------------|---------------|
| Carroll et al. | June 30, 1942 |
| Blake et al.   | July 8, 1947  |
| Cairns et al.  | Feb. 17, 1948 |
| Carroll et al. | Aug. 23, 1955 |
| Carroll        | June 19, 1956 |
| Moessen        | July 31, 1956 |
| Carroll        | Mar. 5, 1957  |